

July 31, 1934.

G. S. EVANS

1,968,753

SOLID DETERGENT

Filed Jan. 26, 1933

3 Sheets-Sheet 1

*Fig. 1.*



INVENTOR

*George S. Evans*  
BY  
*James Louis Martin & Edwards*

ATTORNEYS

July 31, 1934.

**G. S. EVANS**

**1,968,753**

## SOLID DETERGENT

Filed Jan. 26, 1933

3 Sheets-Sheet 2



Fig. 2,

## INVENTOR

BY

BY  
James Harris Morris & Edmonds  
ATTORNEYS

## ATTORNEYS

July 31, 1934.

G. S. EVANS

1,968,753

SOLID DETERGENT

Filed Jan. 26, 1933

3 Sheets-Sheet 3

Fig. 3,



INVENTOR

George S. Evans  
By  
Pennie Davis, Marvin Edmonds

ATTORNEYS

## UNITED STATES PATENT OFFICE

1,968,753

## SOLID DETERGENT

George S. Evans, Bronxville, N. Y., assignor to  
 The Mathieson Alkali Works, Inc., New York,  
 N. Y., a corporation of Virginia

Application January 26, 1933, Serial No. 653,618

8 Claims. (Cl. 87—5)

This invention relates to the manufacture of cakes of detergent material and the invention is particularly concerned with the production of cakes of this character that are especially useful in conditioning the wash water in dish-washing machines. The invention is primarily concerned with the production of detergent cakes which go into solution in water at a substantially constant rate throughout the dissolving period whereby the alkalinity of the wash water can be maintained within a certain desirable range.

In the operation of ordinary dish-washing machines, such as those used in hotels and restaurants, it is customary to add to the re-circulating water quantities of nonforming detergents such as soda ash, caustic soda or tri-sodium phosphate crystals or mixtures of such materials, the detergent compound being added to the water in loose or powder form. The standard dish-washing machine, as adapted to restaurants having a seating capacity up to one hundred and fifty to two hundred, consists of a water tank of approximately fifteen gallon capacity with an overflow outlet, circulating pump, sprays and dish racks, all encased and connected to the water system. Where greater capacity is required, two or three of these machines are employed or machines of larger capacity are used the capacity being in multiples of fifteen gallons. In starting up such a dish-washing machine it is customary first to fill the tank with hot water and then add a charge of the detergent compound. Ordinarily about one-half pound of the chemical is added to a fifteen gallon tank, giving a chemical strength of approximately 233 grains per gallon, and this is supplemented by periodic additions at 15 to 45 minute intervals during the operating period. The fresh water employed for the purpose of rinsing the dishes replaces a portion of the re-circulating water and a corresponding quantity of the re-circulating water is discharged through an overflow pipe, carrying off any solids floating on the surface as well as a portion of the detergent compound. The volume of rinse water added during each cycle of operation is generally equal to one-sixth or one-eighth of the tank capacity so that the volume of tank water is replaced by rinse water with about seven cycles or more of operation. It is thus apparent that the chemical strength of the re-circulating water is rapidly diluted both by consumption in the washing operations and by being carried off in the overflow water.

The quantity of detergent compound required in properly cleansing dishes in the ordinary dish-

washing machine of the type referred to above varies widely depending upon the condition of the dishes being washed and the hardness and temperature of the wash water. For any given conditions there is a limited economic range of chemical strength between the maximum and minimum strengths obtaining when loose or readily soluble detergents are added to the wash water at intervals in accordance with the practice heretofore employed. An alkalinity of between 75 and 150 grains per gallon is usually needed to insure thorough celansing of the dishes under average conditions. An excess of alkali in the re-circulating water is objectionable because of the tendency of the alkali to convert starchy materials into a kind of glue which forms a sticky deposit on the dishes not easily removed by the rinse water. On the other hand, if the alkalinity of the wash water is too low it is necessary to increase materially both the washing and rinsing periods in order to cleanse the dishes thoroughly. The use of detergent material in powder or loose form is objectionable because when a charge of this material is first added the alkalinity of the wash water is excessive and this makes it difficult to cleanse the dishes properly and large quantities of the chemical are soon discharged through the overflow without having performed any useful function. The concentration of the chemical is rapidly reduced until the amount of detergent material in the water is inadequate and another charge of the compound must be added. The alkalinity of the wash water is within the desired range only throughout a relatively small portion of the operating cycle.

One of the objects of the present invention is to provide detergent material in a form such that the efficiency of dish-washing machines and the like may be substantially increased. In general this object is attained by providing cakes or briquettes of detergent material of such configuration and density that the detergent material goes into solution in the dish-washing machine at a rate such that the alkalinity of the wash water remains within the desired range of—say 75 to 150 grains per gallon of wash water throughout a considerable portion of the operating cycle of the machine. In preparing the detergent cakes I prefer to fuse the detergent material and then cast this fused material into cake form, preferably although not necessarily, in a chilled mold which insures the production of cakes of high density. The form of the mold is preferably such as to provide cakes having a ratio of surface area to volume or weight such that the

average solubility rate in circulating water at 120° F. is between 3 and 4½ grams per minute for each 100 square centimeters of original surface area of the cakes. In general, this ratio of area in square centimeters to weight in grams is between .4 and .9, the ratio being preferably limited to between .4 and .5. I prefer to employ metal molds for such molds are capable of absorbing the heat in the fused mass within the mold at a rapid rate with the result that the cast cakes have a high density. Such molds may be referred to as chilled molds and it is to be understood that any type of chilled mold may be employed where high density cakes are desired.

Where the cakes consist essentially of soda ash or mixtures of soda ash and tri-sodium phosphate or soda ash and sodium silicate the best results for the purpose described above are obtained when the cakes are of such size that their weight is between 90 and 600 grams. If cakes of this weight are cast in semi-spherical form, or in any other form having substantially the same ratio of surface area to volume, the average solubility rate of the cakes in circulating water at 120° F. is within a range of 3 to 4½ grams per minute for each 100 square centimeters of original surface area of the cakes. When such cakes are used in the ordinary dish-washing machine having a capacity of 15 gallons the alkalinity of the water is within the range of 75 to 150 grains per gallon throughout the major portion of the total period required for completely dissolving the cakes. By utilizing the present invention it is entirely feasible to maintain the alkalinity of the wash water within the desired range throughout eighty (80%) per cent of the time required for completely dissolving the detergent material, and excessive alkalinity can be avoided at all times.

The characteristics and advantages of my invention will be more apparent upon considering the accompanying drawings of which

Fig. 1 is a graph showing the solubility characteristics of cakes of fused soda ash of various sizes;

Fig. 2 is a graph showing the area per 100 grams and the solubility rate per 100 square centimeters of original surface area of fused soda ash cakes and

Fig. 3 is a graph showing the alkalinity of the wash water in a 15 gallon capacity dish-washing machine, the graph showing the results obtained by the use of one embodiment of the present invention as compared with the use of loose soda ash.

Referring to Fig. 1 of the drawings the several curves represent the alkali content of the wash water in a 15 gallon capacity dish-washing machine operated with a continuous flow of fresh water at the rate of one gallon per minute. The curve A represents the condition obtaining when a charge of 8 ounces or 226½ grams of loose soda ash is added to the 15 gallon tank. This 8 ounce charge was dissolved immediately, as indicated by the small circle at the top of the curve A, giving an alkalinity of somewhat over 230 grains per gallon and during 45 minutes of operation the alkalinity was reduced to below 15 grains per gallon. During the initial portion of this operating cycle the alkalinity of the water was excessive,—considerably more than 150 grains per gallon and the alkalinity was within the desired range of 75 to 150 grains per gallon during a comparatively small portion of the operating period of 45 minutes.

The curves 1 to 6 inclusive of Fig. 1 represent the alkalinity of the wash water when cakes of fused soda ash of various sizes were added to the water, the data for the curves being as follows:—

|             | Grams |
|-------------|-------|
| Curve No. 1 | 90    |
| Curve No. 2 | 232   |
| Curve No. 3 | 415   |
| Curve No. 4 | 642   |
| Curve No. 5 | 1000  |
| Curve No. 6 | 1728  |

The small circle on each curve represents the time at which the fused cake of soda ash was completely dissolved. It will be noted that the total time required for dissolving each of the cakes is substantially the same and that for the cakes weighing more than 600 grams the dissolving rate is excessive during a substantial portion of the dissolving period. This indicates the desirability of limiting the size of the cake to a range within 90 to 600 grams and it will be noted that as to cakes within this range the rate of going into solution is substantially constant throughout the major portion of the period required for the cakes to be completely dissolved. The cakes represented by the curves 1 to 6 of Fig. 1 were cast in an iron mold of semi-spherical shape.

The curves A and B of Fig. 2 represent respectively the surface area in square centimeters per 100 grams for cakes of fused soda ash of the type represented by the curves 1 to 6 of Fig. 1, and the rate of solution of such cakes in grams per 100 square centimeters of surface area per minute. From these curves A and B it will be noted that for the cakes having a weight of 90 grams to 642 grams the rate of solution is within the range of approximately 3 grams per 100 square centimeters of surface area to 4 and 2/3 grams per 100 square centimeters, and it has been found that cakes of fused soda ash, or of mixtures of detergent materials consisting essentially of fused soda ash and tri-sodium phosphate, having this average rate of solution in circulating water at a temperature in the neighborhood of 120° F., provide the desired alkalinity.

In Fig. 3 the curve A represents the alkalinity of the wash water in a 15 gallon capacity dish-washing machine when charges of 226½ grams of loose soda ash are added at 40 minute intervals, and the curve B represents the alkalinity when 226½ gram cakes of fused soda ash are added to the washing machine tank at 40 minute intervals. It will be noted that when the loose soda ash is employed the alkalinity is excessive throughout the initial portion of the cycle and that when the fused cakes of soda ash are used the alkalinity is never in excess of 150 grains per gallon. Furthermore when the fused cakes are employed the alkalinity remains within the desired range of 75 to 150 grains per gallon throughout the major portion of the cycle. The cakes of fused soda ash represented by the curve B of Fig. 3 were made by casting the molten material in metal molds of semi-spherical shape.

The fused cakes of detergent material may consist entirely of soda ash, or of mixtures of soda ash and tri-sodium phosphate and if desired from 1 to 10 per cent by weight of sodium silicate may be added to the mixture, or to the soda ash where no tri-sodium phosphate is used. The soda ash and tri-sodium phosphate may be mixed

in proportions such that the tri-sodium phosphate represents from 10 to 70 per cent by weight and preferably the percentage of tri-sodium phosphate is between 40 and 60 per cent by weight.

5 It is to be understood that my invention is not limited to the specific embodiments thereof illustrated and described but includes such modifications thereof as fall within the scope of the appended claims.

10 I claim:—

1. A fused detergent alkaline salt body in cake form suitable for maintaining the proper degree of alkalinity of the wash water in dish washing machines comprising soda ash as a major ingredient, the said cake having a ratio of surface area in square centimeters to weight in grams between .4 and .9.

2. A fused detergent alkaline salt body in cake form suitable for maintaining the proper degree of alkalinity of the wash water in dish washing machines comprising soda ash as a major ingredient, said cake having a ratio of surface area in square centimeters to weight in grams between .4 and .5.

25 3. A fused detergent alkaline salt body of approximately semi-spherical shape and suitable for maintaining the proper degree of alkalinity of the wash water in dish washing machines comprising soda ash as a major ingredient, said cake having a ratio of surface area in square centimeters to weight in grams between .4 and .9.

35 4. A fused detergent alkaline salt mixture in cake form suitable for maintaining the proper degree of alkalinity of the wash water in dish washing machines comprising as major ingredients soda ash and tri-sodium phosphate blended in proportions such that the tri-sodium phosphate represents 10 to 70 per cent of the total weight of these ingredients, the cake having a ratio of surface area in square centimeters to weight in grams between .4 and .9.

40 5. A fused detergent alkaline salt mixture in

cake form suitable for maintaining the proper degree of alkalinity of the wash water in dish washing machines comprising as major ingredients soda ash and sodium silicate blended in proportions such that the sodium silicate represents 1 to 10 per cent of the total weight of these ingredients, the cake having a ratio of surface area in square centimeters to weight in grams between .4 and .9.

5. A fused detergent alkaline salt mixture in cake form suitable for maintaining the proper degree of alkalinity of the wash water in dish washing machines comprising as major ingredients soda ash and tri-sodium phosphate blended in proportions such that the tri-sodium phosphate represents 40 to 60 per cent of the total weight of these ingredients, the cake having a ratio of surface area in square centimeters to weight in grams between .4 and .9.

6. A fused detergent alkaline salt mixture in cake form suitable for maintaining the proper degree of alkalinity of the wash water in dish washing machines comprising as major ingredients soda ash, tri-sodium phosphate and sodium silicate blended in proportions such that the tri-sodium phosphate represents 10 to 70 per cent of the total weight of soda ash and tri-sodium phosphate and the sodium silicate represents 1 to 10 per cent of the total weight of tri-sodium phosphate and soda ash.

7. A fused detergent alkaline salt body of semi-spherical shape and suitable for maintaining the proper degree of alkalinity of the wash water in dish washing machines comprising soda ash as a major ingredient and having a weight in grams of between 90 and 600 and having an average solubility rate in circulating water at 120 degrees Fahrenheit of between 3 and 4½ grams per minute per 100 square centimeters of original surface area.

115 GEORGE S. EVANS.

45

50

55

60

65

70

75

80

85

90

95

100

105

110

115

120

125

130

135

140

145

150